

## UNITED STATES PATENT OFFICE

KARL SCHRÖTER, OF BERLIN-LICHTENBERG, AND HANS WOLFF, OF BERLIN, GERMANY, ASSIGNORS TO FRIED. KRUPP AKTIENGESELLSCHAFT, OF ESSEN/RUHR, GERMANY

MANUFACTURE OF BODIES FOR TOOLS AND THE LIKE FROM MATERIALS SUCH AS CARBIDES, THE ALLOYS THEREOF, AND THE LIKE

No Drawing. Application filed June 10, 1929, Serial No. 369,913, and in Germany June 15, 1928.

Our invention relates to improvements in the manufacture of bodies for tools and the like from materials such as carbides, the alloys thereof, and the like the working of which by means of tools is difficult by reason of the hardness thereof. As now practised such bodies are made from powdered material by first pressing the same into the desired shape, and thereafter sintering the same. For manufacturing bodies which are less simple in shape, and which therefore cannot be readily pressed into final shape, coherent bodies have been manufactured by first pressing the materials nearly into the desired form, thereafter subjecting the same to preliminary sintering at low temperature for transforming the same into a state allowing working by means of tools, imparting the final shape thereto by cutting tools, and finally subjecting the blank to high sintering. In carrying out this method it is necessary during the preliminary sintering operation to heat the blank exactly at the proper temperature, because when the temperature is not sufficient the body is brittle, and when the temperature is too high the hardness of the blank is such that economical working by means of cutting tools is not possible.

The object of the improvements is to provide a method by means of which bodies of any desired shape can be easily manufactured, and with this object in view our invention consists in forming a hard and rigid body of the desired form from the said powdered material and a suitable binding medium hardening at ordinary temperature or at slightly elevated temperature, thereafter imparting exactly the desired form to the said body by mechanical working, and finally sintering the same at high sintering temperature. The raw material consists of carbides of metals having a high melting point or of mixtures of such carbides with metals having a lower melting point, such for example as iron, cobalt or nickel, and the binding medium may be added to the said material either before or after pressing the same into the desired shape. By adding the said binding medium to the raw material a body is produced which is sufficiently co-

herent to permit working by means of suitable tools in the same way as the bodies heretofore made by the preliminary sintering process. For example, to the hard and rigid body produced by means of the binding medium the desired form, for example sharp cutting edges, can be imparted by mechanical operation. 55

Suitable binding media transforming the powdered raw material into a rigid blank 60 permitting mechanical working are cementing media, resins, lacquer, putties, such as gum arabic, dextrin, shellac, zellon, colophony. Good results have been obtained by adding a 10 to 30% alcoholic solution of shellac to the powdered raw material of high melting point, or by adding the said solution to the body pressed from the said raw material. However, we wish it to be understood that we do not limit ourselves to a binding 65 medium in solution or in suspension in a suitable liquid, and that we may also use a cementing or gluing medium such as shellac or colophony, which is softened at low temperature, or metals or metalloids of low melting point, which matter is added to the powdered raw material of high melting point. When using such materials the body is heated, 70 during or after pressing, at a comparatively low temperature which is not sufficient to 75 cause preliminary sintering, for temporarily transforming the said solid binding medium into a state permitting gluing or cementing of the powdered raw material. The solid body of raw material produced by solidification of the binding medium can be subjected to mechanical working, in the same way as a hard body subjected to preliminary sintering, and more particularly it can be worked 80 by turning, boring, raising, sawing, and filing. By the high sintering process following the mechanical working of the pressed bodies the binding medium is removed, or slight residues remain in the body which do 85 not impair the quality of the final object. 90

The material removed from the blank by mechanical working may be used in the manufacture of other bodies, because it has not been heated at high temperature, so that it 95 100

can be used in the same way as the fresh raw material.

We claim:

1. The herein described method of manufacturing bodies from material such as carbides, alloys thereof, and the like, which consists in producing a body composed of the powdered raw material and a binding medium adapted to bind the powdered raw material into a hard and coherent body, allowing the said body to harden, imparting thereto the desired shape by mechanical working, and thereafter subjecting the same to high sintering temperature.

10 2. The herein described method of manufacturing bodies from material such as carbides, alloys thereof, and the like, which consists in mixing the powdered raw material with a binding medium adapted to transform the same into a hard coherent body, pressing the material and binding medium nearly into the desired form, allowing the same to harden, imparting the final shape to the blank, and heating the same at sintering temperature.

15 3. The herein described method of manufacturing bodies from material such as carbides, alloys thereof, and the like, which consists in pressing the powdered raw material nearly into the desired shape, adding thereto a binding medium adapted to harden with the raw material into a coherent hard body, allowing the raw material and binding medium to harden, imparting the final shape 20 to the blank by mechanical working, and heating the same at sintering temperature.

25 4. The herein described method of manufacturing bodies from material such as carbides, alloys thereof, and the like, which consists in producing a body composed of the powdered raw material and a binding medium in a suitable liquid adapted to bind the powdered raw material into a hard and coherent body, allowing the said body to harden, imparting thereto the desired shape by 30 mechanical working, and thereafter subjecting the same to high sintering temperature.

40 5. The herein described method of manufacturing bodies from material such as carbides, alloys thereof, and the like, which consists in producing a pressed body nearly of the desired final form from the powdered raw material and a powdered solid binding medium adapted to be made soft by heating 45 and to bind the raw material into a hard and coherent body, softening the binding medium and allowing the same to harden again, imparting the final shape to the blank by mechanical working, and heating the same 55 at sintering temperature.

60 6. The herein described method of manufacturing bodies from material such as carbides, alloys thereof, and the like, which consists in producing a body composed of the powdered raw material and a binding me-

dium adapted to bind the powdered raw material into a hard and coherent body, allowing the said body to harden, and thereafter subjecting the same to high sintering temperature.

65 In testimony whereof we hereunto affix our signatures.

KARL SCHRÖTER.  
HANS WOLFF.

70

75

80

85

90

95

100

105

110

115

120

125

130